

J. C. TRAVILLA.

PAVEMENT AND PROCESS FOR MAKING THE SAME.

APPLICATION FILED NOV. 4, 1908.

936,493.

Patented Oct. 12, 1909.

*Fig. 1.*



*Fig. 2.*



*Fig. 4.*



*Fig. 3.*



*Witnesses:*

G. A. Pennington  
Edgar T. Farmer?

*Inventor:*

James C. Travilla,  
By James Davy, Atty.

# UNITED STATES PATENT OFFICE.

JAMES C. TRAVILLA, OF ST. LOUIS, MISSOURI.

## PAVEMENT AND PROCESS FOR MAKING THE SAME.

936,493.

Specification of Letters Patent.

Patented Oct. 12, 1909.

Application filed November 4, 1908. Serial No. 461,051.

*To all whom it may concern:*

Be it known that I, JAMES C. TRAVILLA, a citizen of the United States, and a resident of the city of St. Louis and State of Missouri, have invented a certain new and useful Improvement in Pavements and Processes of Making Same, of which the following is a specification.

My invention relates to pavements and has for its principal objects to provide a resili-  
10 ent, durable, waterproof, dustless and com-  
paratively inexpensive pavement; and to  
provide a simple process of making the same.  
It consists principally in compressing  
15 against a suitable substructure slabs of a bi-  
tuminous mixture of such consistency that  
the material thereof will be forced into the  
interstices in the upper surface of the sub-  
structure and will be spread laterally to  
20 form a continuous layer.

It also consists in the details of construction and in the process of construction hereinafter described and claimed.

In the accompanying drawing, which  
25 forms part of this specification, and wherein  
like symbols refer to like parts wherever  
they occur, Figure 1 is an isometric view,  
partly in cross section, showing a completed  
stone base for my pavement; Fig. 2 is a simi-  
lar view showing the malleable slabs in place  
on said stone base preparatory to their ini-  
tial compression; Fig. 3 is a similar view  
showing the top coating and cross section of  
the pavement before the final compression;  
35 and, Fig. 4 is a fragmentary cross-section of  
the completed pavement.

My pavement comprises a substructure of  
any suitable construction. The substructure  
comprises a base 1 of macadam, telford slag,  
gravel, cinders or other like material. This  
material is suitably bonded and thoroughly  
rolled. Upon this base is a course or layer  
2 of stone, preferably, macadam ranging in  
dimension from one and one half inches to  
45 two and one half inches, which is lightly  
rolled or compressed in position. Over this  
upper layer 2 is spread a thin coating 3 of  
sand or particles of stone or stone dust suf-  
ficient to partially fill the void spaces or in-  
terstices therein. Then a coat 4 of bitumi-  
nous cement is applied over the surface thus  
formed, and previously prepared slabs 5 are  
laid on such cement.

The slabs are made of a lightly compacted  
mixture consisting of bitumen, sand, and  
stone particles and dust in such proportion  
55 that the slab will maintain its shape while  
being handled and transported but will be  
sufficiently soft or plastic to permit it to be  
squeezed into the spaces in the surface of  
the substructure. It is believed to be un-  
necessary to specify any particular composi-  
tion or proportion of ingredients, as the art  
fully discloses how to secure the desired  
qualities. The slabs 5 are laid close to each  
other and are given a preliminary compres-  
sion sufficient to squeeze the material of the  
lower portion thereof into the interstices in  
the upper surface of the substructure. Then,  
a coating 6 of bituminous cement is applied  
70 to the top and sides of the partially com-  
pressed slabs. Before the cement hardens,  
a thin layer 7 of small particles of sharp  
stone, or sand or mineral dust is applied  
thereon, and then the pavement is rolled or  
75 compressed with a heavy roller to the ulti-  
mate extent. By this last rolling operation,  
the following results are produced: The par-  
ticles of stone and sand and dust are forced  
into the bituminous body of the slabs, the  
80 slabs are compressed vertically so that the  
substance thereof completely fills the upper  
interstices of the substructure, they are com-  
pacted to form a hard wearing surface; and  
at the same time, the slabs are spread or  
85 elongated so that the sides thereof are con-  
solidated or welded together to form a sub-  
stantially monolithic layer. In consequence  
of this method of construction, the bitumi-  
nous mixture which originally consisted of a  
90 a multiplicity of slabs becomes ultimately  
a continuous, hard and smooth layer of sub-  
stantially uniform thickness. By reason of  
its being made of portable slabs of uniform  
thickness the application thereof may be  
95 made with the greatest rapidity and assur-  
ance of accuracy, without any particular  
skill; and as the slabs are sufficiently plastic  
at the ordinary atmospheric temperature, it  
is unnecessary to heat them *in situ*, and thus  
100 great economies are effected. By reason of  
the material of the slabs being compressed

2  
into the interstices of the substructure, a strong continuous mechanical interlock is formed between them, which will prevent the creeping of the surface layer and will bind the stone together. The application of the surface coat of cement serves to harden and more effectually waterproof the wearing surface and to coöperate in the welding or coalescence of the abutting ends of the slabs, 5 and the topmost layer of the particles of stone serves to harden and roughen the wearing surface. It is noted, however, that said ton coat of cement and the finish coat of stone particles may both be dispensed with, 10 and that the coat 4 of bituminous cement is 15 also unnecessary.

Obviously, my invention admits of considerable variation from the details hereinbefore specified. For instance, instead of 20 the substructure being formed as hereinbefore described, it may consist of a single thick layer of macadam or it may consist of any other common type of construction. So, too, the slabs may be applied directly to the 25 substructure without the interposition of sand, cement or other substance. Again, the composition of the slabs may be varied as desired, and either the sand, the stone dust or the small stone or particles of stone may 30 be omitted, so long as there is a sufficient aggregate of stony matter. I do not, therefore, wish to restrict myself to the details of construction hereinbefore described.

What I claim is:

35 1. A pavement comprising a substructure and a layer of lightly compacted malleable slabs compressed thereon.

2. A pavement comprising a substructure of macadam and a layer of lightly compacted malleable slabs of bituminous mixture 40 compressed into the interstices thereof.

3. A pavement consisting of a substructure and a layer of lightly compacted malleable slabs of bituminous mixture compressed thereon, said substructure comprising a base of macadam and a layer of coarse 45 macadam thereon.

4. A pavement consisting of a substructure and a layer of malleable slabs of bituminous mixture compressed thereon, said substructure comprising a base of macadam and a layer of coarser macadam thereon, and sand and stone screenings partially filling the interstices of said coarser layer.

5. A pavement consisting of a substructure, a layer of malleable slabs compressed thereon, and a coat of bituminous cement between them, said substructure comprising a base of macadam, a layer of coarse macadam thereon, and sand and stone screenings partially filling the interstices of said coarser layer.

6. A pavement consisting of a substructure, a layer of malleable slabs of bituminous

65 mixture compressed thereon, a coat of bituminous cement between said substructure and said slabs, a coat of bituminous cement on said slabs and a thin layer of small particles of stone dust or sand compressed into said slabs.

7. A pavement consisting of a substructure, a layer of malleable slabs of bituminous mixture compressed thereon, a coat of bituminous cement between said substructure and said slabs, a coat of bituminous cement 75 on said slabs and a thin layer of small particles of stone compressed into said slabs, said substructure comprising a base of macadam, a layer of coarse macadam thereon, and sand partially filling the interstices of 80 said finer layer.

8. A pavement comprising a substructure having a rough upper surface and a layer of malleable slabs compressed into the interstices of such surface, said slabs consisting 85 of a mixture of bitumen, sand and stone dust shaped with slight pressure so as to render the finished slabs malleable at ordinary temperature.

9. The process of building a pavement 90 which consists in forming a substructure, applying thereto lightly compacted malleable slabs and compressing said slabs into the surface interstices of such substructure.

10. The process of building a pavement 95 which consists in forming a base of macadam and a layer of coarse macadam, and applying thereto lightly compacted malleable slabs of bituminous mixture and compressing said slabs into the interstices in said 100 upper layer.

11. The process of building a pavement which consists in forming a substructure, coating the same with bituminous cement, applying lightly compacted malleable slabs 105 on said cement, and compressing said slabs into the surface interstices of such substructure.

12. The process of building a pavement which consists in forming a base of macadam 110 and a layer of coarser macadam thereon, partially filling the interstices of said upper layer with sand or stone particles and then applying a coat of bituminous cement and then applying malleable slabs of bituminous 115 mixture and compressing said slabs to fill the interstices in said upper layer.

13. The process of building a pavement which consists of forming a suitable substructure, coating the same with bituminous 120 cement, applying malleable slabs on said cement, partially compressing said slabs, then coating the partially compressed slabs with bituminous cement and covering the same with small particles of stone, and then 125 rolling the surface to compress and spread said slabs into a continuous layer.

14. The process of building a pavement

which consists in forming a base of macadam and a layer of coarser macadam thereon and partially filling the interstices of said upper layer with sand or stone particles,  
5 coating the surface thus formed with bituminous cement and then applying malleable slabs of bituminous mixture on said cement, partially compressing said slabs, then coating the partially compressed slabs with  
10 bituminous cement and covering the same

with small particles of stone, and then rolling the surface further to compress said slabs and spread them into a continuous layer.

Signed at St. Louis, Missouri, November 2, 15  
1908.

JAS. C. TRAVILLA.

Witnesses:

JAMES A. CARR,  
J. B. MEGOWN.